# EUROPEAN PATENT APPLICATION

(11) **EP 4 787 391 A1**
(43) Date of publication of application: **05.08.2026**
(21) Application number: 26155995.9
(22) Date of filing: 03.02.2026
(51) Int. Cl.: G21H 1/06

(54) **ISOTOPE BATTERY AND METHOD OF FABRICATING THE SAME**

(30) Priority: 04.02.2025 KR 20250013666; 02.02.2026 KR 20260020827
(71) Applicant: LG Energy Solution, Ltd., Seoul 07335 (KR)
(72) Inventor: SHIN, Dae Beom, 34122 Daejeon (KR); KIM, Dong Myung, 34122 Daejeon (KR); KIM, Je Young, 34122 Daejeon (KR); SHIN, Dong Myung, 34122 Daejeon (KR); CHOI, Hee Jo, 34122 Daejeon (KR); SEO, Ji Hyeok, 34122 Daejeon (KR)
(74) Representative: BCKIP Part mbB

(57) **Abstract**

Disclosed herein is an isotope battery (1, 1a, 1b, 1c, 1d) and its fabrication method. The isotope battery (1, 1a, 1b, 1c, 1d) comprises a first conductivity type semiconductor layer (110a), a radiation source (130) provided on a first side surface of the first conductivity type semiconductor layer (110a) and having at least partially a droplet shape, and a second conductivity type semiconductor layer (120a) facing the first side surface of the first conductivity type semiconductor layer (110a) with the radiation source (130) in-between. The isotope battery (1, 1a, 1b, 1c, 1d) of the present disclosure and its fabrication method may be mass-produced by a simple process without wasting expensive materials.

## Description

### [Technical Field]

The present disclosure relates to an isotope battery and a method of fabricating the same, and more particularly to an isotope battery and a method of fabricating the same that can be mass-produced in a simple process without wasting expensive materials.

### [Background]

The radiation emitted by the radioactive isotope can be absorbed through the surface of the p-n junction semiconductor and converted into electrical energy. The radiation generates electron-hole pairs in the space-charge region of the p-n junction semiconductor, and the generated carriers have voltage-current characteristics. Nuclear battery units utilizing these properties have the advantage of being able to supply power stably for a long period of time. Since radiation sources that emit radiation are very expensive materials, methods to reduce unnecessary waste are required.

### [Prior Art Document]

### [Patent Document]

(Patent Document 1) Chinese Published Patent No. 104051042

### [Summary]

### [Technical Problem]

The inventive concept provides an isotope battery that can be mass-produced in a simple process without wasting expensive materials.

The inventive concept provides a method of fabricating an isotope battery that can be mass-produced in a simple process without wasting expensive materials.

### [Technical Solution]

According to an aspect of the inventive concept, there is provided an isotope battery comprising a first conductivity type semiconductor layer, a radiation source provided on a first side surface of the first conductivity type semiconductor layer and having at least partially a droplet shape, and a second conductivity type semiconductor layer facing the first side surface of the first conductivity type semiconductor layer with the radiation source in-between.

In some embodiments, the first side surface of the first conductivity type semiconductor layer is a flat surface.

In some embodiments, the radiation source has a contact angle with the flat surface of the first conductivity type semiconductor layer greater than 90 degrees.

In some embodiments, the radiation source has a contact angle with the flat surface of the first conductivity type semiconductor layer less than 90 degrees.

In some embodiments, the first conductivity type semiconductor layer has a concave pit, wherein the radiation source is buried in the pit and protrudes from the pit.

In some embodiments, the radiation source has at least a partially ellipsoid surface.

In some embodiments, the radiation source has a contact angle greater than 90 degrees with a flat surface of the first conductivity type semiconductor layer.

In some embodiments, an additional second conductivity type semiconductor layer is provided on a second side surface of the first conductivity type semiconductor layer opposite the first side surface.

In some embodiments, the first conductivity type semiconductor layer has a substantially constant thickness.

In some embodiments, an additional first conductivity type semiconductor layer is provided on a side surface of the second conductivity type semiconductor layer and faces the second side surface of the first conductivity type semiconductor layer with the radiation source in-between.

In some embodiments, a photon generating layer is provided between the radiation source and the first side surface of the first conductivity type semiconductor layer

In some embodiments, the radiation source comprises an ellipsoid surface, wherein the photon generating layer embeds the radiation source and covers the ellipsoid surface.

According to another aspect of the inventive concept, there is provided a method of fabricating an isotope battery, comprising the steps of preparing a radiation source slurry comprising a radiation source, distributing the radiation source slurry in the form of droplets on a first side surface of a first conductivity type semiconductor layer of a semiconductor substrate, curing the radiation source slurry distributed in the form of droplets, and forming a second conductivity type semiconductor layer on the cured radiation source and the first side surface of the first conductivity type semiconductor layer.

According to embodiments, in the step of distributing the radiation source slurry in the form of droplets, the radiation source slurry is discharged onto the first side surface of the first semiconductor layer of the semiconductor substrate in the form of droplets having a diameter of about 10 µm to about 10 mm.

According to embodiments, in the step of distributing the radiation source slurry in the form of droplets, the radiation source slurry is ejected from a nozzle in the form of droplets, whereafter the droplets are seated on the semiconductor substrate.

According to embodiments, the viscosity of the radiation source slurry is from about 0.5 cP to about 2000 cP at 25°C.

### [Advantageous Effects]

The isotope battery of the present disclosure and its fabrication method have the effect of being able to be mass-produced in a simple process without wasting expensive materials.

The effects of the exemplary embodiments of the present disclosure are not limited to those mentioned above, and other effects not mentioned may be clearly derived and understood by one having ordinary knowledge in the technical field to which the exemplary embodiments of the present disclosure belong from the following description. In other words, unintended effects of practicing the exemplary embodiments of the present disclosure may also be derived from the exemplary embodiments of the present disclosure by one having ordinary knowledge in the technical field.

### [Brief Description of the Drawings]

FIG. 1 is a side view illustrating an isotope battery according to an embodiment of the present disclosure.
FIGS. 2a to 2d are schematic plan views illustrating the placement of a radiation source in an isotope battery according to embodiments of the present disclosure.
FIG. 3 is a side view illustrating an isotope battery with a contact angle θ less than 90 degrees.
FIGS. 4a, 4b, 4c and FIGS. 5 and 6 are side views illustrating isotope batteries according to other embodiments of the present disclosure.
FIG. 7a and 7b are schematic plan views illustrating the shape and arrangement of radiation sources in an isotope battery according to embodiments of the present disclosure.
FIG. 8 is a flow diagram illustrating a method of fabricating an isotope battery according to an embodiment of the present disclosure.
FIGS. 9a through 9d are schematic side views illustrating a step-by-step method of fabricating an isotope battery.
FIG. 10 is a flow diagram illustrating a method of manufacturing an isotope battery according to the embodiment described with reference to FIG. 4a.
FIGS. 11a to 11e are schematic side views illustrating a step-by-step method of manufacturing an isotope battery according to another embodiment.

### [Best Mode for Carrying out the Invention]

Hereafter, the preferred embodiments of the concept of the present disclosure will be described in detail with reference to the accompanying drawings. However, the embodiments of the concept of the present disclosure may be modified in various other forms, and the scope of the concept of the present disclosure should not be construed as being limited to the embodiments described below. It is desirable that the embodiments of the concept of the present disclosure be construed as being provided to more fully explain the concept of the present disclosure to a person with average knowledge in the industry. The same symbols mean the same elements throughout. Furthermore, the various elements and areas in the drawings are depicted schematically. Therefore, the concept of the present disclosure is not limited by the relative sizes or spacings depicted in the accompanying drawings.

The terms 'first,' 'second,' etc. may be used to describe various components, but the components are not limited by the terms. The terms are used only to distinguish one component from another. For example, the first component may be named the second component and vice versa, without falling outside the scope of the rights of the concept of the present disclosure.

The terms used in this application are used merely to describe specific embodiments and are not intended to limit the concept of the present disclosure. Singular expressions include plural expressions unless the context clearly indicates otherwise. In this application, the expressions 'comprising' or 'having' are to be understood as designating the presence of features, numbers, steps, actions, components, sub-components, or combinations thereof as described in the specification, but not as precluding the existence or addition of one or more other features, numbers, actions, components, sub-components, or combinations thereof.

Unless otherwise defined, all terms used herein, including technical terms and scientific terms, have the same meaning as commonly understood by a person of ordinary skill in the technical field to which the concept of the present disclosure belongs. It will also be understood that terms that are commonly used and defined in dictionaries should be interpreted as having a meaning consistent with their meaning in the context of the relevant technology, and should not be interpreted in an overly formal sense unless explicitly defined here.

In the event that a different embodiment is otherwise possible, a specific process sequence may be performed differently from the sequence described. For example, two processes described in succession may be performed substantially simultaneously, or in the reverse order of the sequence described.

In the accompanying drawings, for example, variations of the shapes shown may be expected depending on the manufacturing technology and/or tolerances. Therefore, the embodiments of the present disclosure should not be construed as being limited to the specific shapes of the areas shown in the specification, but should include, for example, changes in shape caused by the manufacturing process. All terms used herein 'and/or' include each of the components mentioned and all combinations of one or more of them. In addition, the term 'substrate' used in this specification may refer to the substrate itself or a laminated structure including a predetermined layer or film formed on the substrate and its surface. In addition, the term 'surface of the substrate' in this specification may refer to the exposed surface of the substrate itself or the outer surface of a predetermined layer or film formed on the substrate.

It will be understood that when an element such as a layer, film, region, or substrate is referred to as being "above" or "on" another element, it can be directly on the other element or intervening elements may also be present.

Furthermore, relative terms, such as "lower" or "bottom" and "upper" or "top," may be used herein to describe one element's relationship to another element as illustrated in the Figures. It will be understood that relative terms are intended to encompass different orientations of the device in addition to the orientation depicted in the Figures. For example, if the device in one of the figures is turned over, elements described as being on the "lower" side of other elements would then be oriented on "upper" sides of the other elements. The term "lower," can therefore, encompasses both an orientation of "lower" and "upper," depending on the particular orientation of the figure. Similarly, if the device in one of the figures is turned over, elements described as "below" or "beneath" other elements would then be oriented "on" or "above" the other elements. The terms "below" or "beneath" can, therefore, encompass both an orientation of above and below.

### (First embodiment)

FIG. 1 is a side view illustrating an isotope battery 1 according to one embodiment of the present disclosure. FIG. 2a is a schematic plan view illustrating the arrangement of radiation sources 130 in the isotope battery 1 according to an exemplary embodiment of the present disclosure.

Referring to FIGS. 1 and 2a, the isotopic battery 1 comprises a first conductivity type semiconductor layer 110a having a first (upper) side surface and a second (lower) side surface opposite the first side surface. Radiation sources 130 may be disposed on the first side surface of the first conductivity type semiconductor layer 110a. The radiation sources 130 may have at least a partial droplet shape. As used herein, the term 'droplet shape' may refer to the shape of a free curved surface that a fluid having any surface tension and viscosity may assume. The term 'partial' means that not all the surface of the droplet will be curved depending on where the droplet is placed. For example, when the droplet is placed on the first side surface of the first conductivity type semiconductor layer 110a, a part of the otherwise curved surface is flat when the droplet comes into contact with the first side surface of the semiconductor layer 110a.

FIG. 2a shows an example placement of the radiation sources, where the radiation sources 130 are arranged in a grid at regular spacings, but the present disclosure is not limited to this. In some embodiments, the radiation sources 130 may be randomly disposed on the first conductivity type semiconductor layer 110a.

In some embodiments, when a substantially round droplet (see the droplet 130s in FIG. 9b to be described below) is placed (dropped) onto the first side surface of the first conductivity type semiconductor layer 110a, such that the radiation source 130 comes into contact with a flat portion of the first side surface of the first conductivity type semiconductor layer 110a, a portion of the radiation source 130 in contact with the flat portion of the first side surface of the first conductivity type semiconductor layer 110a becomes substantially flat due to the specific weight of the radiation source 130 whilst the remainder portion of the surface of the radiation source 130 remains curved. In some embodiments, this remainder portion of the surface of the radiation source 130 may have an ellipsoid shape.

In some embodiments, the radiation source 130 may include a radioactive isotope that emits beta rays. For example, the radiation source 130 may include one or more selected from the group consisting of tritium (³H, tritium), calcium-45 (⁴⁵Ca), nickel-63 (⁶³Ni), copper-67 (⁶⁷Cu), strontium-90 (⁹⁰Sr), promethium-147 (¹⁴⁷Pm), osmium-194 (¹⁹⁴OS), thulium-171 (¹⁷¹Tm), thallium-204 (²⁰⁴TI), tantalum-182 (¹⁸²Ta), cadmium-115 (¹¹⁵Cd), cadmium-113 (¹¹³Cd), germanium-75 (⁷⁵Ge), cerium-141 (¹⁴¹Ce), cerium-144 (¹⁴⁴Ce), and tungsten-185 (¹⁸⁵W). However, the present disclosure is not limited to these.

In some embodiments, the radiation source 130 may include a radioactive isotope that emits alpha rays. For example, the radiation source 130 may include one or more selected from the group consisting of americium-241 (²⁴¹Am), americium-243 (²⁴³Am), polonium-209 (²⁰⁹Po), polonium-210 (²¹⁰Po), plutonium-238 (²³⁸Pu), plutonium-239 (²³⁹Pu), curium-240 (²⁴⁰Pu), plutonium-238 (²³⁸Pu), plutonium-239 (²³⁹Pu), curium-242 (²⁴²Cm), curium-244 (²⁴⁴Cm), curium-249 (²⁴⁹Cm), promethium-147 (¹⁴⁷Pm), uranium-238 (²³⁸U), thorium-232 (²³²Th), radium-226 (²²⁶Ra), bismuth-210 (²¹⁰Bi), neptunium-237 (²³⁷Np), europium-152 (¹⁵²Eu), francium-223 (²²³Fr), astatine-210 (²¹⁰At), protactinium-231 (²³¹Pa), einsteinium-253 (²⁵³Es), californium-252 (²⁵²Cf), and berkelium-249 (²⁴⁹Bk). However, the present disclosure is not limited to these.

In some embodiments and as shown in FIG. 1 (and also FIG. 3), the radiation source 130 may be in contact with the first side surface of the first conductivity type semiconductor layer 110a at a predetermined contact angle θ. In some embodiments, the contact angle θ may be greater than 90 degrees (as shown in FIG. 1). In some other embodiments, the first side surface of the first conductivity type semiconductor layer 110a may be a substantially flat surface, and the radiation source 130 may have a contact angle θ with the first side surface of the first conductivity type semiconductor layer 110a greater than 90 degrees (as also shown in FIG. 1).

As shown in FIG. 1 and FIG. 3, the contact angle is defined as the angle between the first side surface of the first semiconductor layer 110a and the tangent to the curved surface of the radiation source at the contact point of the curved surface of the radiation source with the first side surface of the first semiconductor layer 110a.

In FIG. 1, the first side surface of the first semiconductor layer 110a is illustrated as a flat surface. However, the first side surface may not be necessarily completely flat and those of ordinary skill in the art would understand the contact angle of the radiation source (droplets) can also be defined for the droplets at the contact point between the curved surface of the radiation source droplet and the first non-flat surface. That is, the contact angle is defined by an angle between a line tangential to the radiation source 130 and a line tangential to the first semiconductor layer 110a at the contact point of the curved surface of the radiation source 130 with the first side surface of the first semiconductor layer 110a.

In some embodiments, the contact angle θ of the radiation source 130 with the first side surface of the first conductivity type semiconductor layer 110a may be from about 100 degrees to about 160 degrees. In some other embodiments, the contact angle θ of the radiation source 130 with the first side surface of the first conductivity type semiconductor layer 110a may range from about 100 degrees to about 160 degrees, from about 105 degrees to about 155 degrees, from about 110 degrees to about 150 degrees, from about 115 degrees to about 145 degrees, from about 120 degrees to about 140 degrees, from about 125 degrees to about 135 degrees, or any two of these values.

FIG. 2b is a schematic plan view illustrating an arrangement of radiation sources 130 in the isotope battery 1 according to another embodiment of the present disclosure.

The radiation sources 130 may be arranged with any predetermined regularity. In some embodiments, as shown in FIG. 2b, the radiation sources 130 may be arranged so that their respective centers are located at the vertices of a series of imaginary equilateral triangles (which are schematically indicated in FIG. 2b with the solid lines connecting the radiation sources 130).

By arranging the radiation sources 130 so that their centers are located at the vertices of the imaginary equilateral triangles, the number of radiation sources 130 that can be accommodated per unit area can be maximized.

FIG. 2c is a schematic plan view illustrating an arrangement of radiation sources 130 in the isotope battery 1 according to yet another embodiment of the present disclosure.

Referring to FIG. 2c, each center of the radiation sources 130 may be arranged to be located at a vertex of an imaginary isosceles triangle arranged in a row. As in FIG. 2b, each center of the radiation source 130 may not necessarily be located at the vertex of a series of imaginary equilateral triangles arranged in a row.

In some embodiments, the triangles in which each center of the radiation source 130 is disposed may be triangles having some different shapes. Accordingly, the radiation sources 130 may be arranged somewhat irregularly.

FIG. 2d is a schematic plan view illustrating an arrangement of radiation sources 130 in the isotope battery 1 according to still another embodiment of the present disclosure.

Referring to FIG. 2d, the radiation sources 130 may be randomly disposed on the first conductive type semiconductor layer 110a. In some embodiments, the number density of the radiation sources 130 per unit area of the first conductive type semiconductor layer 110a may be substantially constant from location to location.

In some other embodiments, the contact angle θ may be less than 90 degrees. FIG. 3 is a side view of another example illustrating an isotope battery 1a in which the contact angle θ is less than 90 degrees. As in FIG. 1, also in FIG. 3, the first side surface of the first conductivity type semiconductor layer 110a may be a substantially flat surface, and the radiation source 130 may have a contact angle θ with the first side surface of the first conductivity type semiconductor layer 110a that is less than 90 degrees.

In some embodiments, the contact angle θ that the radiation source 130 has with the first conductivity type semiconductor layer 110a may be from about 20 degrees to about 80 degrees. In some embodiments, the contact angle θ of the radiation source 130 with the first conductivity type semiconductor layer 110a may have a range between about 20 degrees to about 80 degrees, about 25 degrees to about 75 degrees, about 30 degrees to about 70 degrees, about 35 degrees to about 65 degrees, about 40 degrees to about 60 degrees, about 45 degrees to about 55 degrees.

As will be discussed below in more detail with reference to FIG: 8, the radiation source 130 may be formed by placing a radiation source slurry having a predetermined viscosity (and specific weight) on the substrate 10 in the form of droplets. The droplets of the radiation source slurry disposed on the substrate 10 will be seated on the substrate 10 at a predetermined contact angle θ depending on one or more of the surface tension (or specific weight), viscosity, wetting property with the first side surface of the first semiconductor layer 110a, and the like. For example, if the surface tension and/or viscosity of the droplets of the radiation source slurry is relatively high, the contact angle θ may be greater than 90 degrees. Conversely, if the surface tension and/or viscosity of the droplets of the radiation source slurry is relatively low, the contact angle θ may be smaller than 90 degrees.

For another example, if the wetting property of the droplets of the radiation source slurry with the substrate 10 is relatively high, the contact angle θ may be smaller than 90 degrees. Conversely, if the droplets of the radiation source slurry have a relatively low wetting property with the substrate 10, the contact angle θ may be greater than 90 degrees.

Referring to FIGS. 1 to 3, the first conductivity type semiconductor layer 110a may be a layer doped with dopants of a first conductivity type of the substrate 10, that is the layer 110a is a layer portion of the substrate 10 in which the dopant of the first conductivity type is doped in a certain concentration. The layer 120b is a layer portion of the substrate 10 in which the dopant of the second conductivity type is doped in a certain concentration.

In some embodiments, the first conductivity type semiconductor layer 110a may have a substantially constant thickness.

The base material of the substrate 10 (i. e. of the layers 110a and 120b of which the dopant concentrations are different from each other according to the conductivity type) may include, for example, a group III-V semiconductor material. The III-V group semiconductor material may include InAIP, InGaP, InAlGaP, ZnSe, AlAs, AlAsP, or yttria-stabilized zirconia (YSZ).

In some embodiments, the base material of the substrate 10 may include a diamond substrate, a SiC substrate, a GaN substrate, a Bi₂O₃/GeO₂ substrate, a Sm₂O₃/Bi₂O₃/GeO₂ substrate, a Sm₂O₃/Bi₂O₃/B₂O₃ substrate, a Sm₂O₃/Bi₂O₃/GeO₂/B₂O₃ substrate, a sapphire substrate, or a combination thereof, which may be an undoped substrate.

In some other embodiments, the base material of substrate 10 may include a diamond substrate, a SiC substrate, a GaN substrate, a Bi₂O₃/GeO₂ substrate, a Sm₂O₃/Bi₂O₃/GeO₂ substrate, a Sm₂O₃/Bi₂O₃/B₂O₃ substrate, a Sm₂O₃/Bi₂O₃/GeO₂/B₂O₃ substrate, a sapphire substrate, or a combination thereof, which may be doped with dopants.

In some other embodiments, the base material of the substrate 10 may have the formula AMO₃ (where A is one or more selected from the group consisting of La, Ba, Sr, and K, and M is one or more selected from the group consisting of Al, In, Ga, Ti, Sn, Hf, Ta, and Zr).

Specifically, the base material of the substrate 10 may include one or more selected from the group consisting of BaSnO₃, BaHfO₃, BaZrO₃, BaHf₁₋ₓTiₓO₃(where 0<x<1), Ba₁₋ₓLaₓSnO₃(where 0<x<1), Bi₄Ge₃O₁₂, Al₂O₃, Y₂O₃, La₂O₃, Ga₂O₃, Bi₂O₃, ZrO₂, HfO₂, Ta₂O₅, TiO₂, LaInO₃, LaGaO₃, SrZrO₃, SrHfO₃, SrTaO₇, LaIn₁₋ₓGaₓO₃(where 0<x<1), LaGaO₃, SrTiO₃, KTaO₃, HfSiO₄, Ta₃Ti₂Oₓ, and LaAlO₃ (where 0<x<1).

In some embodiments, the substrate 10 may include a semiconductor substrate. In some embodiments, the substrate 10 may include a non-conductor substrate.

In some embodiments, the first conductivity type semiconductor layer 110a may include a metal oxide having a bandgap energy of 2.7 eV or greater. In some embodiments, the metal oxide may have the formula AMO₃ (where A is one or more selected from the group consisting of La, Ba, Sr, and K, and M is one or more selected from the group consisting of Al, In, Ga, Ti, Sn, Hf, Ta, and Zr).

Specifically, the metal oxide is selected from the group consisting of BaSnO₃, BaHfO₃, BaZrO₃, BaHf₁₋ₓTiₓO₃(where 0<x<1), Ba₁₋ₓLaₓSnO₃(where 0<x<1), Bi₄Ge₃O₁₂, Al₂O₃, Y₂O₃, La₂O₃, Ga₂O₃, Bi₂O₃, ZrO₂, HfO₂, Ta₂O₅, TiO₂, LaInO₃, LaGaO₃, SrZrO₃, SrHfO₃, SrTaO₇, LaIn₁₋ₓGaₓO₃(where 0<x<1), LaGaO₃, SrTiO₃, KTaO₃, HfSiO₄, Ta₃Ti₂Oₓ, and LaAlO₃ (where 0<x<1).

The metal oxide is not only stable in high temperature and high humidity environments, but also has a high mobility of carriers, which can efficiently absorb radiation emitted by the radiation source 130 to provide high energy conversion efficiency. In addition, there is no inelastic collision in the carrier movement, which is favorable for energy loss and heat dissipation. For example, the metal oxide may have a high carrier mobility of 45 cm²/(V·s) or more, 80 cm²/(V·s) or more, 120 cm²/(V·s) or more, or even 300 cm²/(V·s) or more.

Metal oxides are materials that can be doped with both types of conductivity (n or p) and have the advantage of being able to provide high current or high voltage depending on the direction of the applied bias.

As also shown in FIG. 1 and FIG. 3, the isotope battery 1 may further include a second conductivity type semiconductor layer 120a covering the first (upper) side surface of first conductivity type semiconductor layer 110a and the radiation source 130.

In some embodiments and as illustrated in FIG. 1 and FIG. 3, the second conductivity type semiconductor layer 120a may be in contact with an ellipsoid surface of the radiation source 130. In some embodiments, the second conductivity type semiconductor layer 120a may be partially in contact with the first side surface of the first conductivity type semiconductor layer 110a.

In some embodiments, the second conductivity type semiconductor layer 120a may be a layer doped with dopants of a second conductivity type.

The base material of the second conductivity type semiconductor layer 120a may employ the base material described above with respect to the first conductivity type semiconductor layer 110a. In some embodiments, the base material of the second conductivity type semiconductor layer 120a may be the same as the base material of the first conductivity type semiconductor layer 110a. In some other embodiments, the base material of the second conductivity type semiconductor layer 120a may be different from the base material of the first conductivity type semiconductor layer 110a.

In some embodiments, the first conductivity type semiconductor layer 110a may be doped with dopants of the first conductivity type. The second conductivity type semiconductor layer 120a may be doped with dopants of a second conductivity type different from the first conductivity type. The first conductivity type semiconductor layer 110a and second conductivity type semiconductor layer 120a may generate electron-hole pairs by radiation emitted by the radiation source 130.

In some embodiments, the dopant of the first conductivity type may be an n-type dopant and the dopant of the second conductivity type may be a p-type dopant. In some other embodiments, the dopant of the first conductivity type may be a p-type dopant and the dopant of the second conductivity type may be an n-type dopant. One of ordinary skill in the art will understand that depending on the conductivity type of the dopants doped in each region or layer, one of the first conductivity type semiconductor layer 110a and the second conductivity type semiconductor layer 120a may act as a cathode and the other may act as an anode. That is, if the dopant of the first conductivity type is an n-type dopant and the dopant of the second conductivity type is a p-type dopant, the first conductivity type semiconductor layer 110a may act as an anode and the second conductivity type semiconductor layer 120a may act as a cathode.

Conversely, if the dopant of the first conductivity type is a p-type dopant and the dopant of the second conductivity type is an n-type dopant, the first conductivity type semiconductor layer 110a may act as a cathode and the second conductivity type semiconductor layer 120a may act as an anode.

The n-type doped region may be a semiconductor region doped with, for example, nitrogen (N), phosphorus (P), arsenic (As), or antimony (Sb), which are 15^{th} group elements of the periodic table, or it may be a compound semiconductor doped with nitrogen (N), phosphorus (P), arsenic (As), or antimony (Sb), which are 15^{th} group elements of the periodic table. As used herein, a compound semiconductor refers to a semiconductor composed of two or more elements and may be, for example, silicon carbide, silicon oxide, aluminum phosphide (AlP), aluminum arsenide (AlAs), gallium arsenide (GaAs), or gallium nitride (GaN).

The p-type dopant-doped region may be a semiconductor region or a semiconductor layer doped with, for example, boron (B), aluminum (Al), gallium (Ga), or indium (In), or a compound semiconductor doped with boron (B), aluminum (Al), gallium (Ga), or indium (In), which are 13^{th} group elements of the periodic table.

In some embodiments, the first conductivity type semiconductor layer 110a and/or the second conductivity type semiconductor layer 120a may include an organic material used in organic layers that receive light to generate power, such as in solar cell applications. For example, the first conductivity type semiconductor layer 110a and/or the second conductivity type semiconductor layer 120a may include a thiophene-like compound. Alternatively, the first conductivity type semiconductor layer 110a and/or the second conductivity type semiconductor layer 120a may be an inorganic-organic hybrid type by appropriately mixing the aforementioned inorganic and organic materials.

In some embodiments, a depletion region may be formed near the interface where the first conductivity type semiconductor layer 110a and the second conductivity type semiconductor layer 120a contact each other.

In some embodiments, an additional second conductivity type semiconductor layer 120b may be provided below the first conductivity type semiconductor layer 110a. In some embodiments, the additional second conductivity type semiconductor layer 120b may be made of substantially the same material as the second conductivity type semiconductor layer 120a disposed on the upper part of the first conductivity type semiconductor layer 110a.

In some embodiments, an additional first conductivity type semiconductor layer 110b may be provided on the upper part of the second conductivity type semiconductor layer 120a. In some embodiments, the additional first conductivity type semiconductor layer 110b may be made of substantially the same material as the first conductivity type semiconductor layer 110a the first (upper) side surface of which is covered by the second conductivity type semiconductor layer 120a.

As shown in FIG. 3, the isotope battery 1 may also include a first electrode 105a and a second electrode 105b capable of transmitting generated electrical energy to the outside.

As also shown in FIG. 3, the first electrode 105a may be coupled to the first conductivity type semiconductor layer 110a and the additional first conductivity type semiconductor layer 110b. The second electrode 105b may be coupled to the second conductivity type semiconductor layer 120a and the additional second conductivity type semiconductor layer 120b.

The first electrode 105a and the second electrode 105b are not particularly limited in type, size, shape, etc. as long as they are electrically conductive without causing physical and chemical changes in the isotope battery 1. For example, the first electrode 105a and the second electrode 105b may be cylindrical, tetrahedral, hexahedral, torus, or pad-shaped. In some embodiments, the first electrode 105a and the second electrode 105b each independently include a metallic material such as gold (Au), silver (Ag), platinum (Pt), stainless steel, copper (Cu), aluminum (Al), nickel (Ni), or titanium (Ti), include transparent oxides such as fluorine (F)-doped tin oxide (FTO) or indium tin oxide (ITO, In₂O₃/SnO₂), or include carbon-based compounds such as carbon-nanotubes, graphene, or graphene oxide.

### (Second embodiment)

FIG. 4a is a side view illustrating an isotope battery 1b according to another embodiment of the present disclosure. The isotope battery 1b shown in FIG. 4a differs in that a concave pit P is formed in the first conductivity type semiconductor layer 110a compared to the isotope battery 1a shown in FIG. 3, and is otherwise substantially the same. Therefore, the following description will focus on this difference.

Referring to FIG. 4a, the isotope battery 1b may be provided with a concave pit P in the first conductivity type semiconductor layer 110a. At least a part of the radiation source 130 may be disposed in the pit 130. The cross-sectional shape of the pit P is not particularly limiting. In some embodiments, the pit P may have a concave surface with a curved inner surface. In some embodiments, the concave surface of the pit P may be part of a spherical surface or part of an ellipsoid surface.

As shown in FIG. 4a, in some embodiments, the radiation source 130 may be provided at least partially within the pit P and protrude outside of the pit P. In some other embodiments, the radiation source 130 may also partially extend over a part of the flat first (upper) side surface of the first conductivity type semiconductor layer 110a adjacent to the pit P.In some still other embodiments, the radiation source 130 may be fully buries inside the pit P

In the embodiments, where the radiation source 130 also extends over the flat first (upper) side surface of the first conductivity type semiconductor layer 110a adjacent to the pit P, the upper surface of the radiation source 130 above the first (upper) side surface of the first conductivity type semiconductor layer 110a may be curved. In some embodiments, the radius of curvature of the upper surface of the radiation source 130 may be greater than the radius of curvature of the lower surface of the radiation source 130 in the pit P.

In some embodiments, the radiation source 130 may have a droplet shape that completely fills the pit P. The residual portion of the radiation source 130 above the pit that remains after filling the pit P may have a droplet shape.

Similarly to the above description with reference to FIG. 3 (showing the angle θ which the radiation source 130 forms with the first (upper) side surface of the first conductivity type semiconductor layer 110a without the provision of pits P, also when pits P are provided therein, the radiation source 130 may be in contact with the flat first side (upper) side surface of the first conductivity type semiconductor layer 110a forming a predetermined contact angle θ therewith. In some embodiments, this contact angle θ may be less than 90 degrees. In FIG. 4a, the contact angle θ is shown to be less than 90 degrees, but one of ordinary skill in the art will understand that the contact angle θ may be greater than 90 degrees. One of ordinary skill in the art will understand that the contact angle θ may depend on the surface tension, viscosity, and wetting property of the radiation source slurry with the first conductivity type semiconductor layer 110a in which or on which the radiation source 130 is formed.

As already described above, in some embodiments, the first conductivity type semiconductor layer 110a may have a substantially constant thickness. As shown in FIG. 4a, also when pits P are formed in the first conductivity type semiconductor layer 110a, the first conductivity type semiconductor layer 110a may have a substantially constant thickness also in the portion forming the pit P.

Referring to FIG. 4b, the entirety of the radiation source 130 may be provided within the pit P. That is, the entirety of the radiation source 130 may be embedded within the pit P. In some embodiments, the radiation source 130 may be completely embedded in the pit and may not protrude outside of the pit. In some embodiments, the upper surface of the radiation source 130 may be in the same plane as the flat upper surface of the first conductive type semiconductor layer 110a.

In some embodiments, the lower surface of the second conductive type semiconductor layer 120a may have a flat surface and may be in contact with the upper surface of the first conductive type semiconductor layer 110a and the upper surface of the radiation source 130.

Referring to FIG. 4c, the pit P may have concave sides, i.e., the pit P may have a width in the horizontal direction that increases and then decreases with distance from the lower surface of the second conductive type semiconductor layer 120a. In some embodiments, a radiation source 130 accommodated within the pit P may have a maximum width in the horizontal direction at a height about midway between itself and the pit P.

The radiation source 130 shown in FIG. 4c may be entirely embedded within the pit P, as may the radiation source 130 shown in FIG. 4b. In some embodiments, the radiation source 130 may be completely embedded in the pit P and may not protrude outside of the pit P. In some embodiments, the upper surface of the radiation source 130 may be in the same plane as the flat upper surface of the first conductive type semiconductor layer 110a.

In some embodiments, the lower surface of the second conductive type semiconductor layer 120a may have a flat surface and may be in contact with the upper surface of the first conductive type semiconductor layer 110a and the upper surface of the radiation source 130.

### (Third embodiment)

FIG. 5 is a side view illustrating an isotope battery 1c according to yet another embodiment of the present disclosure. The isotope battery 1c shown in FIG. 5 differs from the isotope battery 1 shown in FIG. 1 in that the above mentioned additional first conductivity type semiconductor layer 110b is positioned on the first side (upper) side surface of the first conductivity type semiconductor layer 110a and the radiation source 130, and the above mentioned second conductivity type semiconductor layer 120a is disposed on the additional first conductivity type semiconductor layer 110b. Otherwise the structure is substantially the same as in FIG. 1. Accordingly, the following description will focus on this difference.

Referring to FIG. 5, the radiation source 130 is provided on the first (upper) side surface of the first conductivity type semiconductor layer 110a as in FIG. 1, and the additional first conductivity type semiconductor layer 110b is provided on the parts of the first (upper) side surface of the first conductivity type semiconductor layer 110b not covered by the radiation source 130 and covers at least a part of the of the radiation source 130. In some embodiments, the radiation source 130 may be completely covered by the additional first conductivity type semiconductor layer 110b.

### (Fourth embodiment)

FIG. 6 is a side view illustrating an isotope battery 1d according to another embodiment of the present disclosure. The isotope battery 1d shown in FIG. 6 differs from the isotope battery 1 in FIG. 1 in that it further includes a photon generating layer 140. Accordingly, the following description will focus on on the contruction of the isotope battery 1d including such a photon generating layer 140.

Referring to FIG. 6, the isotope battery 1d further includes a photon generating layer 140 inside of which the radiation source 130 is provided (embedded).

In some embodiments, the photon generating layer 140 may include a first photon generating layer 140a and a second photon generating layer 140b. In some embodiments, the first photon generating layer 140a may be disposed on the first conductivity type semiconductor layer 110a, the second photon generating layer 140b may be disposed on the first photon generating layer 140a, and the radiation source 130 may be provided on the first photon generating layer 140a. The second photon generating layer 140b is provided on parts of the first photon generating layer 140a not covered by the radiation source 130, and covers the radiation source 130 provided thereon. The second conductivity type semiconductor layer 120a is provided on the second photon generating layer 140b, and the additional first conductivity type semiconductor layer 110b is provided on the second conductivity type semiconductor layer 120a as in FIG. 1.

The photon generating layer 140 may be any material layer capable of emitting photons in response to radiation particles emitted from the radiation source 130.

For example, the photon generating layer 140 may employ materials such as, but not limited to, Ba₂Ca(BO₃)₂, BaHfO₃, BaI₂:Ce, BeO, BaF₂, BaMgF₄, Cs₂LiLuCi₆:Ce, K₂YF₅, KCaF₃, YI₃:Ce, and the like. Various examples of such photon generating layers 140 are disclosed at https://scintillator.lbl.gov/inorganic-scintillator-library/.

The photon generating layer 140 may emit photons in response to alpha rays incident from the radiation source 130. The photons generated by the photon generating layer 140 may be incident on the junction region between the first conductive type semiconductor layer 110a, 110b and the second conductive type semiconductor layer 120a, 120b, and electrical energy may be generated by the photons.

The radiation source 130 may be disposed on the first photon generating layer 140a having a substantially flat surface. The radiation source 130 may be in contact with the first photon generating layer 140a at a predetermined contact angle θ. In some embodiments, the contact angle θ may be greater than 90 degrees. In some embodiments, the first photon generating layer 140a is a substantially flat surface, and the radiation source 130 may have a contact angle θ with the first conductivity type semiconductor layer 110a greater than 90 degrees.

In some embodiments, the contact angle θ of the radiation source 130 with the first photon generating layer 140a may be from about 100 degrees to about 160 degrees. In some embodiments, the contact angle θ of the radiation source 130 with the first photon generating layer 140a can range from about 100 degrees to about 160 degrees, about 105 degrees to about 155 degrees, about 110 degrees to about 150 degrees, about 115 degrees to about 145 degrees, about 120 degrees to about 140 degrees, about 125 degrees to about 135 degrees, or any two of these values.

In some other embodiments, the contact angle θ may be less than 90 degrees.

In some embodiments, the first photon generating layer 140a is a substantially flat surface, and the radiation source 130 may have a contact angle θ with the first photon generating layer 140a that is less than 90 degrees.

In some embodiments, the contact angle θ that the radiation source 130 has with the first photon generating layer 140a may be from about 20 degrees to about 80 degrees. In some embodiments, the contact angle θ of the radiation source 130 with the first photon generating layer 140a may have a range of about 20 degrees to about 80 degrees, about 25 degrees to about 75 degrees, about 30 degrees to about 70 degrees, about 35 degrees to about 65 degrees, about 40 degrees to about 60 degrees, about 45 degrees to about 55 degrees, or any two of these values.

The second photon generation layer 140b provided on the first photon generation layer 140a may be made of substantially the same material as the first photon generating layer 140a. In some embodiments, the second photon generating layer 140b may be disposed between the radiation source 130 and the second conductivity type semiconductor layer 120a such that it fully embeds the radiation source 130.

In some embodiments, the radiation source 130 may be disposed between the first photon generating layer 140a and the second photon generating layer 140b. In some embodiments, the radiation source 130 may be provided on the first photon generating layer 140a and the second photon generating layer 140b may be provided on the first photon generating layer 140a embedding the radiation source 130. In some embodiments, the radiation source 130 may face the first conductivity type semiconductor layer 110a with the first photon generating layer 140a in-between. In some embodiments, the radiation source 130 may face the second conductivity type semiconductor layer 120a with the second photon generating layer 140b in-between.

The second photon generating layer 140b may at least partially cover a droplet-shaped surface of the radiation source 130. In some embodiments, the second photon generating layer 140b may completely cover the droplet-shaped surface of the radiation source 130.

In some embodiments, a clear cut interface may exist between the first photon generating layer 140a and the second photon generating layer 140b, that is the first photon generating layer 140a and the second photon generating layer 140b are separate layers which abut at each other. In some embodiments, the presence of an interface between the first photon generating layer 140a and the second photon generating layer 140b may not be measurable or visible. In some embodiments, there may be gradual transition between the first photon generating layer 140a and the second photon generating layer 140b.

In some embodiments, the second conductivity type semiconductor layer 120a may be provided on the second photon generating layer 140b. In some embodiments, the second conductivity type semiconductor layer 120a may have a substantially constant thickness.

Above the second conductivity type semiconductor layer 120a, the additional first conductivity type semiconductor layer 110b may be provided.

In FIG. 6, the second conductivity type semiconductor layer 120a is shown as being provided on top of the second photon generating layer 140b, and the additional first conductivity type semiconductor layer 110b is shown as being provided on top of the second conductivity type semiconductor layer 120a.

However, one of ordinary skill in the art will understand that the stacking order of these layers may be reversed. In some embodiments, the additional first conductivity type semiconductor layer 110b may be provided on top of the second photon generation layer 140b, and the second conductivity type semiconductor layer 120a may be provided on top of the first conductivity type semiconductor layer 110b. In this case, the connection relationship of the electrodes 105a, 105b may be modified accordingly such that the electrodes 105a, 105b are connected to the same layers as described above.

### (Fifth embodiment)

FIGS. 7a and 7b are schematic plan views illustrating the shape and arrangement of the radiation source 130 in an isotope battery according to embodiments of the present disclosure.

Referring to FIG. 7a, the radiation sources 130 may have the form of predetermined spaced lines rather than droplets. The radiation source 130 may have the form of two or more lines extending substantially parallel onto the first conductive type semiconductor layer 110a. However, the radiation sources 130 may still contact the first conductive type semiconductor layer 110a with a contact angle θ as shown in FIGS. 1 and 3.

The spacing between the radiation sources 130 may be greater than the width of the radiation sources 130. In some embodiments, the spacing between the radiation sources 130 may be from about 3 times to about 20 times the width of the radiation sources 130.

Referring to FIG. 7b, the radiation source 130 may have the form of a plurality of lines extending in directions that intersect each other. In some embodiments, the radiation source 130 may have the form of a plurality of lines extending in a first direction and a plurality of lines extending in a second direction intersecting the first direction. In some embodiments, the first direction and the second direction may be perpendicular to each other. However, the present disclosure is not limited to this, and the first direction and the second direction may intersect at any angle such that they are not parallel to each other.

The radiation sources 130 extending in the first direction may extend substantially in parallel and may take the form of lines spaced apart at predetermined spacings. The radiation sources 130 extending in the second direction may also extend substantially parallel and may take the form of lines spaced apart at predetermined spacings.

The radiation sources 130 extending in the first direction and the radiation sources 130 extending in the second direction may still have a contact angle θ as shown in FIGS. 1 and 3 and may contact the first conductive type semiconductor layer 110a.

### (Sixth embodiment)

FIG. 8 is a flow diagram illustrating a method of fabricating an isotope battery 1 according to one embodiment of the present disclosure. FIGS. 9a to 9d are schematic side views illustrating a step-by-step method of fabricating the isotope battery 1 according to one embodiment of the present disclosure.

Referring to FIGS. 8 and 9a, a radiation source slurry including a radiation source is prepared (S10).

The radiation source slurry may include a radiation source and a dispersant capable of dispersing the radiation source and imparting fluidity to the radiation source. The type and content of the dispersant may be determined by considering the viscosity, surface tension and wetting property with the surface of the respective layer on which the radiation source is to be provided.

The radiation source has been described with reference to FIG. 1 and will not be described in detail herein. The dispersant can be, but is not limited to, any solvent having a suitable viscosity and capable of dispersing the radiation source. In some embodiments, the dispersant is a chlorinated solvent such as chloroform, methylene chloride, 1,2-dichloroethane, 1,1,2-trichloroethane, chlorobenzene, o-dichlorobenzene; an ether-based solvent such as tetrahydrofuran, dioxane; an aromatic hydrocarbon-based solvent such as toluene, xylene, trimethylbenzene, cresol; aliphatic hydrocarbon solvents such as cyclohexane, methylcyclohexane, n-pentane, n-hexane, n-heptane, n-octane, n-nonane, n-decane; ketone solvents such as acetone, methyl ethyl ketone, cyclohexanone; ester solvents such as ethyl acetate, butyl acetate, ethyl cellosolve acetate; polyhydric alcohols and their derivatives, including ethylene glycol, ethylene glycol monobutyl ether, ethylene glycol monoethyl ether, ethylene glycol monomethyl ether, dimethoxyethane, propylene glycol, diethoxymethane, triethylene glycol monoethyl ether, glycerin, and 1,2-hexanediol; alcohol-based solvents, such as methanol, ethanol, propanol, isopropanol, cyclohexanol; sulfoxide-based solvents, such as dimethylsulfoxide; amide-based solvents, such as N-methyl-2-pyrrolidone, N,N-dimethylformamide; benzoate-based solvents, such as butylbenzoate, methyl-2-methoxybenzoate; tetralin; and 3-phenoxytoluene. In some embodiments, the dispersion medium may be one of the above solvents alone, or a mixture of two or more solvents.

In some embodiments, the radiation source slurry may have a viscosity of from about 0.5 cP to about 2000 cP at 25°C. In some embodiments, the radiation source slurry may have a viscosity of from about 0.5 cP to about 2000 cP at 25 °C, from about 0.7 cP to about 1800 cP, about 1 cP to about 1500 cP, about 3 cP to about 1300 cP, about 5 cP to about 1000 cP, about 8 cP to about 900 cP, about 10 cP to about 800 cP, about 13 cP to about 700 cP, about 15 cP to about 600 cP, about 18 cP to about 500 cP, about 20 cP to about 400 cP, about 30 cP to about 350 cP, about 50 cP to about 300 cP, about 80 cP to about 250 cP, about 100 cP to about 200 cP, about 130 cP to about 150 cP, or a range between any two of these figures.

If the viscosity of the radiation source slurry is too small, it may be difficult to form droplets. If the viscosity of the radiation source slurry is too large, it may be difficult to manufacture due to poor processability.

In addition, a substrate 10 is prepared to distribute the radiation source slurry thereon.

The substrate 10 may include the first conductivity type semiconductor layer 110a and the second conductivity type semiconductor layer 120b. In FIG. 9a, the first conductivity type semiconductor layer 110a is shown as having a flat upper surface, but the present disclosure is not limited to this. In some embodiments, the first conductivity type semiconductor layer 110a may have a pit P as shown in FIGS. 4a to 4c.

The first conductivity type semiconductor layer 110a and the second conductivity type semiconductor layer 120b have been described with reference to FIGS. 1 to 3, and therefore will not be described in detail herein.

Referring to FIGS. 8 and 9b, the previously prepared radiation source slurry 130s may be distributed in droplet form 130s on the first conductivity type semiconductor layer 110a (S20).

In some embodiments, the radiation source slurry may be provided on the substrate 10 via a nozzle 5. The radiation source slurry may be ejected from the nozzle 5 in the form of droplets 130s. In some embodiments, when the radiation source slurry is ejected from the nozzle 5 in the form of a droplet 130s, the droplet 130s may be at least momentarily free-surfaced with respect to the entire surface area of the droplet. That is, the droplet may completely break away from the nozzle 5 prior to contact with the substrate 10. The droplets 130s may then be seated on the substrate 10.

The droplets 130s that have escaped from the nozzle 5 may have a diameter of from about 10 µm to about 10 mm. In some embodiments, the droplet 130s may have a diameter of about 10 µm to about 10 mm, about 20 µm to about 8 mm, about 50 µm to about 5 mm, about 80 µm to about 4 mm, about 100 µm to about 3 mm, about 200 µm to about 2 mm, about 300 µm to about 1 mm, about 500 µm to about 800 µm, about 600 µm to about 700 µm, or a range between any two of these figures.

If the droplets 130s are too small or too large in diameter, it may be difficult to distribute them in droplet form on the substrate 10.

In some other embodiments, droplets 130s of the radiation source slurry may contact the substrate 10 before fully exiting the nozzle 5.

If the viscosity and/or surface tension of the radiation source slurry droplets 130s is relatively high, the contact angle θ may be greater than 90 degrees. Conversely, if the viscosity and/or surface tension of the radiation source slurry 130s is relatively low, the contact angle θ may be less than 90 degrees.

Referring to FIGS. 8 and 9c, the radiation source slurry distributed in the form of droplets 130s may be cured (S30).

The radiation source slurry droplets 130s can be cured by removing dispersion medium present in the radiation source slurry droplets 130s. In some embodiments, the dispersion medium may be removed by heating. In some embodiments, the dispersion medium may be removed by depressurization. In some embodiments, the dispersion medium may be removed by heating and depressurization. However, the method of curing the radiation source slurry droplets 130s is not limited to removing the dispersion medium, and one of ordinary skill in the art will understand that the radiation source slurry 130s can be cured in a variety of ways depending on the nature of the dispersion medium. For example, the radiation source slurry 130s may be cured by crosslinking the dispersion medium.

Referring to FIGS. 8 and 9d, the second conductivity type semiconductor layer 120a is formed on the cured radiation source 130 (S40).

In some embodiments, the second conductivity type semiconductor layer 120a may be made of substantially the same material as the additional second conductivity type semiconductor layer 120b disposed on the lower part of the first conductivity type semiconductor layer 110a.

The additional first conductivity type semiconductor layer 110b may then be formed on top of the second conductivity type semiconductor layer 120a. In some embodiments, the additional first conductivity type semiconductor layer 110b may be made of substantially the same material as the first conductivity type semiconductor layer 110a.

The additional first conductivity type semiconductor layer 110b and the second conductivity type semiconductor layer 120a may each be independently formed by a variety of methods, including, but not limited to, chemical vapor deposition (CVD), physical vapor deposition (PVD), atomic layer deposition (ALD), epitaxial growth, and the like.

Then, although not shown in FIG. 8 and FIG: 9, the first electrode 105a and the second electrode 105b may be formed to provide the isotope battery 1 as shown in FIG. 1.

### (Seventh embodiment)

FIG. 10 is a flow diagram illustrating a method of manufacturing an isotope battery 1b according to the embodiment described with reference to FIG. 4a. FIGS. 11a to 11e are schematic side views illustrating a step-by-step method of manufacturing the isotope battery 1b.

Referring to FIGS. 10 and 11a, a radiation source slurry including a radiation source is prepared and a pit P is formed on the second conductive type semiconductor layer 120b (step P10).

Since the preparation of the radiation source slurry has been described above with reference to FIG. 8, a detailed description is omitted here.

The pit P may be formed by forming an etch mask on the second conductive type semiconductor layer 120b, and selectively etching the second conductive type semiconductor layer 120b using the etch mask. Specifically, the pit P may be formed by selectively removing a portion of the second conductive type semiconductor layer 120b exposed through the etch mask.

Selective removal of the second conductive type semiconductor layer 120b may be performed by methods known to those of ordinary skill in the art, such as wet etching, dry etching, sputtering, and the like.

The etch mask may then be removed.

Referring to FIGS. 10 and 11b, a first conductive type semiconductor layer 110a may be formed (step P20). In some embodiments, the first conductive type semiconductor layer 110a may be formed by implanting ions of opposite conductivity type onto the top surface of the second conductive type semiconductor layer 120b. Injecting ions of the opposite conductivity type into the upper surface of the second conductive type semiconductor layer 120b at a sufficient concentration may result in the formation of the first conductive type semiconductor layer 110a having the first conductivity type on the upper surface of the second conductive type semiconductor layer 120b.

In some other embodiments, the first conductive type semiconductor layer 110a may be formed by deposition on an upper surface of the second conductive type semiconductor layer 120b. For example, the first conductive type semiconductor layer 110a may be formed on the upper surface of the second conductive type semiconductor layer 120b by methods such as chemical vapor deposition, physical vapor deposition, epitaxial growth, and the like.

Referring to FIGS. 10 and 11c, the previously prepared radiation source slurry 130s may be distributed in the form of droplets on the first conductive type semiconductor layer 110a (step P30).

In some embodiments, the radiation source slurry 130s may be provided onto the pit P via a nozzle 5. The radiation source slurry 130s may be ejected from the nozzle 5 in the form of droplets. The nozzle 5 may be configured to remember or detect the position of the pit P and spray droplets of the radiation source slurry 130s at that position.

In some embodiments, when the radiation source slurry 130s is ejected from the nozzle 5 in the form of a droplet, the droplet may be at least momentarily free-surfaced with respect to the entire surface area of the droplet. That is, the droplet may completely break away from the nozzle 5 prior to contact with the pit P and form a free surface like a sphere or ball under its surface tension. The droplet may then be seated on the pit P.

The droplet seated on the pit P may be embedded within the pit P. The droplets may enter the pit P by pressure exerted by the nozzle 5 and/or by capillary action exerted by the pit P. In some embodiments, a portion of the droplet may completely bury the pit P and the remainder of the droplet may have a free surface protruding above the pit P.

Referring to FIGS. 10 and 11d, the radiation source slurry 130s distributed in the form of droplets may be cured (step P40). This has been described with reference to FIGS. 8 and 9c and will not be described in detail here.

Referring to FIGS. 10 and 11e, a second conductive type semiconductor layer 120a may be formed on the cured radiation source 130 (step P50).

In some embodiments, the second conductive type semiconductor layer 120a may be made of substantially the same material as the second conductive type semiconductor layer 120b disposed on the lower part of the first conductive type semiconductor layer 110a.

An additional first conductive type semiconductor layer 110b may then be formed on top of the second conductive type semiconductor layer 120a. In some embodiments, the first conductive type semiconductor layer 110b may be made of substantially the same base material as the first conductive type semiconductor layer 110a.

The first conductive type semiconductor layer 110b and the second conductive type semiconductor layer 120a may each be independently formed by a variety of methods, including, but not limited to, chemical vapor deposition (CVD), physical vapor deposition (PVD), atomic layer deposition (ALD), epitaxial growth, and the like.

Subsequent formation of the first electrode 105a and second electrode 105b may result in the isotope battery 1b shown in FIG. 4a.

Although embodiments of the present disclosure have been described in detail above, one of ordinary skill in the art to which the present disclosure belongs will be able to make many modifications to the present disclosure without departing from the spirit and scope of the present disclosure as defined in the appended claims. Accordingly, future modifications on the embodiments of the present disclosure will not depart from the art of the present disclosure.

### [Description of Reference Numerals]

1, 1a, 1b, 1c, 1d: ISOTOPE BATTERY
5: NOZZLE
10: SUBSTRATE
105a: FIRST ELECTRODE
105b: SECOND ELECTRODE
110a: FIRST CONDUCTIVITY TYPE SEMICONDUCTOR LAYER
110b: ADDITIONAL FIRST CONDUCTIVITY TYPE SEMICONDUCTOR LAYER
120a: SECOND CONDUCTIVITY TYPE SEMICONDUCTOR LAYER
120b: ADDITIONAL SECOND CONDUCTIVITY TYPE SEMICONDUCTOR LAYER
130: RADIATION SOURCE
130s: DROPLET OF RADIATION SOURCE SLURRY
140: PHOTON GENERATING LAYER
140a: FIRST PHOTON GENERATING LAYER
140b: SECOND PHOTON GENERATING LAYER

## Claims

1. An isotope battery (1, 1a, 1b, 1c, 1d), comprising:
a first conductivity type semiconductor layer (110a);
a radiation source (130) provided on a first side surface of the first conductivity type semiconductor layer (110a) and having at least partially a droplet shape; and
a second conductivity type semiconductor layer (120a) facing the first side surface of the first conductivity type semiconductor layer (110a) with the radiation source (130) in-between.

2. The isotope battery (1, 1a, 1b, 1c, 1d) of claim 1, wherein
the first side surface of the first conductivity type semiconductor layer (110a) is a flat surface.

3. The isotope battery (1, 1a, 1b, 1c, 1d) of claim 2, wherein
the radiation source (130) has a contact angle with the flat surface of the first conductivity type semiconductor layer (110a) greater than 90 degrees.

4. The isotope battery (1, 1a, 1b, 1c, 1d) of claim 2, wherein
the radiation source (130) has a contact angle with the flat surface of the first conductivity type semiconductor layer (110a) less than 90 degrees.

5. The isotope battery (1, 1a, 1b, 1c, 1d) of claim 1, wherein
the first conductivity type semiconductor layer (110a) has a concave pit (P), wherein
the radiation source (130) is buried in the pit (P) and protrudes from the pit (P).

6. The isotope battery (1, 1a, 1b, 1c, 1d) of claim 5, wherein
the radiation source (130) has at least a partially ellipsoid surface.

7. The isotope battery (1, 1a, 1b, 1c, 1d) of claim 5, wherein
the radiation source (130) has a contact angle greater than 90 degrees with a flat surface of the first conductivity type semiconductor layer (110a).

8. The isotope battery (1, 1a, 1b, 1c, 1d) of claim 1, further comprising:
an additional second conductivity type semiconductor layer (120b) on a second side surface of the first conductivity type semiconductor layer (110a) opposite the first side surface.

9. The isotope battery (1, 1a, 1b, 1c, 1d) of claim 8, wherein
the first conductivity type semiconductor layer (110a) has a substantially constant thickness.

10. The isotope battery (1, 1a, 1b, 1c, 1d) of claim 8, further comprising:
an additional first conductivity type semiconductor layer (110b) on a side surface of the second conductivity type semiconductor layer (120a) and facing the second side surface of the first conductivity type semiconductor layer (110a) with the radiation source in-between.

11. The isotope battery (1, 1a, 1b, 1c, 1d) of claim 1, further comprising:
a photon generating layer (140, 140a, 140b) between the radiation source (130) and the first side surface of the first conductivity type semiconductor layer (110a).

12. The isotope battery (1, 1a, 1b, 1c, 1d) of claim 11, wherein
a surface of the radiation source (130) facing the second conductivity type semiconductor layer (120a) comprises an ellipsoid surface, wherein
the photon generating layer (140, 140a, 140b) extends onto the ellipsoid surface of the radiation source (130) and covers the ellipsoid surface.

13. A method of fabricating an isotope battery (1, 1a, 1b, 1c, 1d), comprising:
preparing (S10) a radiation source slurry (130s) comprising a radiation source (130);
distributing (S20) the radiation source slurry (130s) in the form (130s) of droplets (130s) on a first side surface of a first conductivity type semiconductor layer (110a, 110b) of a semiconductor substrate (10);
curing (S30) the radiation source slurry (130s) distributed in the form (130s) of droplets (130s); and
forming (S40) a second conductivity type semiconductor layer (120a) on the cured radiation source (130) and the first side surface of the first conductivity type semiconductor layer (110a).

14. The method of fabricating an isotope battery (1, 1a, 1b, 1c, 1d) of claim 13, wherein
in the step (S20) of distributing the radiation source slurry (130s) in the form (130s) of droplets (130s), the radiation source slurry (130s) is discharged onto the first side surface of the first semiconductor layer (110a) of the semiconductor substrate (10) in the form of droplets (130s) having a diameter of about 10 µm to about 10 mm.

15. The method of fabricating an isotope battery (1, 1a, 1b, 1c, 1d) of claim 13, wherein
in the step (S20) of distributing the radiation source slurry (130s) in the form of droplets (130s), the radiation source slurry (130s) is ejected from a nozzle in the form of droplets (130s), wherein the ejected droplets form a free surface with respect to the total surface area, and whereafter the droplets (130s) are seated on the semiconductor substrate (10).

16. The method of fabricating an isotope battery (1, 1a, 1b, 1c, 1d) of claim 13, wherein
the viscosity of the radiation source slurry (130s) is from about 0.5 cP to about 2000 cP at 25°C.
